

## UNITED STATES PATENT OFFICE

2,560,371

## SULFUR-HALOGEN COMPOUND

Harry W. Rudel, Roselle Park, N. J., assignor to  
Standard Oil Development Company, a corpora-  
tion of Delaware

No Drawing. Original application December 29,  
1945, Serial No. 638,433. Divided and this ap-  
plication October 20, 1948, Serial No. 55,641

3 Claims. (Cl. 260—293.4)

1

The present invention relates to sulfur-halo-  
gen compounds and particularly to the reaction  
products of thiocarbamates and halogenated hy-  
drocarbons which have utility as extreme pres-  
sure additives for lubricating oils, and other uses  
in hydrocarbon polymers such as natural and  
synthetic rubbers, and the like. This applica-  
tion is a division of my copending application  
Serial No. 638,433, filed December 29, 1945, now  
Patent No. 2,491,772 dated December 20, 1949, 10  
which claims an extreme pressure lubricant.  
The present invention relates to a composition  
per se which forms an active ingredient of such  
a lubricant.

In the prior art, various additives have been  
suggested to improve the film strength of min-  
eral lubricating oils. Among the many E. P.  
additives heretofore recommended, those hydro-  
carbon derivatives containing both active halo-  
gen and active sulfur have proved themselves to  
be very effective in increasing the loadbearing  
characteristics of mineral lubricating oil. Even  
though these sulfur-halogen compounds are ex-  
ceedingly successful as E. P. additives, many of  
them have one characteristic which detracts  
from their acceptability. This characteristic is  
that these sulfur-halogen compounds tend to be  
somewhat unstable during storage, especially at  
temperatures above 100° F., liberating a hydro-  
halogen acid which is corrosive to metal con-  
tainers. Such sulfur-halogen compounds are  
frequently too corrosive for use with certain  
types of bearings. Attempts have been made to  
overcome this excessive corrosiveness of sulfur-  
halogen compounds by the use of inhibitors but  
without much success. While the use of in-  
hibitors is somewhat successful in delaying the  
appearance of evidence of the corrosiveness of  
sulfur-halogen E. P. additives, they are often  
objectionable for the reason that they react  
with the additive or its decomposition products  
to give insoluble precipitates. Such reaction  
both detracts from the quality of the E. P. ad-  
ditive and destroys the inhibitor.

An object of the present invention is the pro-  
duction of a novel, less corrosive type of sulfur-  
halogen compound. Another object is an im-  
provement in E. P. lubricants. These and other  
objects will be apparent to those skilled in the art  
upon reading the following description.

The present invention is based upon the dis-  
covery that the reaction product of a chlorinated  
hydrocarbon containing active chlorine and an  
alkali metal salt of alkyl or aryl dithiocarbamic  
acid, which may also be designated as alkyl or

2

aryl-substituted alkali metal dithioaminofor-  
mate, is an oil-soluble compound having the  
property in oil solution of increasing the load-  
bearing characteristics of a mineral lubricating  
oil, and is stable during storage and relatively  
non-corrosive to metals. This reaction is illus-  
trated by the following equation:



wherein R is an alkyl, cycloalkyl, aryl, aralkyl  
or alkaryl radical such as methyl, ethyl, propyl,  
amyl; cyclopentyl, cyclohexyl, or phenyl, benzyl,  
xylyl, etc. or a heterocyclic nitrogen-containing

radical, such as piperidine; R' is hydrogen or a  
hydrocarbon radical such as alkyl, cycloalkyl,  
aryl, aralkyl, alkaryl, etc.; R'' is a hydrocarbon  
residue derived from a petroleum mineral oil  
distillate such as paraffin wax, kerosene and aro-  
matic petroleum fractions having from 8 to 30  
carbon atoms to the molecule; Met is an alkali  
metal such as sodium, potassium, lithium, etc.;  
Hal is one of the halogens such as chlorine, bro-  
mine or iodine, of which chlorine is preferred  
and x is a positive number of sufficient magni-  
tude that the weight per cent of halogen in the  
compound  $RHal_x$  will range between 5 and 50%,  
preferably 30-40%, the final reaction product  
containing 5 to 40%, preferably 25 to 35% by  
weight of halogen. The value of x will there-  
fore normally range between 2 and 5. The re-  
action may be carried out in the presence of a  
ketone solvent such as methyl ethyl ketone or  
acetone, although any other organic solvent, ex-  
cept alcohol, which is capable of dissolving the  
carbamate, may be used, and at the reflux tem-  
perature of the particular solvent employed.  
After the reaction is complete, which generally  
requires from 1-3 hours, the reaction mixture is  
filtered to remove inorganic salts, after which  
the solvent is recovered by distillation and the  
product is refiltered to remove any residual in-  
organic salts that may be present.

The halogenated hydrocarbon represented by  
R''Hal\_x which may be a halogenated paraffin wax,  
kerosene or aromatic petroleum fraction is made  
by halogenating the hydrocarbon selected until  
on a weight percentage basis the halogen con-  
tent of the halogenated hydrocarbon ranges from  
about 5% to as much as 50%. One example of  
a suitable halogenated hydrocarbon is one made  
by chlorinating kerosene to a chlorine content  
of about 40%, by passing chlorine through kero-  
sene at atmospheric pressure and a temperature  
of about 155°-200° F. for 3 hours. The time

3 required to sufficiently chlorinate a petroleum mineral oil distillate under these conditions of temperature and pressure will range from about 30 minutes to 5 hours. Within the range specified, the chlorine content of the chlorinated hydrocarbon may be varied to accommodate any previously determined sulfur-chlorine requirements in the final product.

The alkali metal salt of the hydrocarbon substituted dithiocarbamic acid is made by reacting a primary or secondary amine, carbon disulfide and alkali metal hydroxide according to the following equation:



In this formula the radicals R and R' possess the same designations as were ascribed to R and R' in the preceding formula illustrating the reaction between the carbamate salt and the halogenated hydrocarbon. The reaction is carried out by suspending stoichiometric amounts of amine and caustic in a solvent such as methyl ethyl ketone, which suspension is then cooled in an ice bath or other equivalent cooling means, and carbon disulfide is then added slowly with agitation. Since the reaction is exothermic, the carbon disulfide must be added cautiously so as to maintain the reactants at a low temperature and prevent undue volatilization of the carbon disulfide. In view of the fact that carbon disulfide is a highly volatile liquid, some excess, up to about 10% over that theoretically required, may be used without any harmful effects, for the purpose of compensating for any carbon disulfide lost through volatilization.

The substituted dithiocarbamic halogenated esters, containing from about 2 to 10% of sulfur and preferably 25 to 35% of chlorine, resulting from the reaction between the alkali metal salt of the substituted dithiocarbamic acid and the chlorinated hydrocarbon can then be blended in amounts ranging from 2 to 30% by weight, based on the total composition, preferably about 10%, in a mineral lubricating oil to yield an extreme pressure lubricant. In compounding such an extreme pressure lubricant, any of the numerous types of low pour point lubricating oils may be used; it is preferred, however, to use a Pennsylvania type oil having a viscosity in the range of from about 50 to about 150 seconds S. U. V. at 210° F. and a cold test below 0° F. The following examples will serve to illustrate specific embodiments of the invention:

#### EXAMPLE 1

20 parts by weight sodium hydroxide  
42.6 parts by weight piperidine  
43.2 parts by weight carbon disulfide  
407 parts by weight chlorinated kerosene containing 39.8% of chlorine

The sodium hydroxide in powdered form was suspended in 250 cc. of methyl ethyl ketone in a reactor equipped with a stirrer and the piperidine was then added, after which the mixture was chilled in an ice bath. The carbon disulfide was then added dropwise and the addition of the carbon disulfide was accompanied by a vigorous exothermic reaction, yielding, after the reaction had subsided, a heavy yellow suspension of sodium piperidyl dithioformate in the solvent. The chlorinated kerosene and 250 cc. additional methyl ethyl ketone were placed in a separate reactor equipped with a reflux condenser; the heavy yellow suspension was then added to the chlorinated kerosene in methyl ethyl ketone and the

whole refluxed for 2 hours. The reaction mixture was then cooled and filtered to remove sodium chloride and the filtrate distilled under a reduced pressure of 37 mm. to remove the methyl ethyl ketone. The residue from the distillation was again filtered to take out any last traces of sodium chloride. 435 parts by weight of a product containing 4.9% sulfur and 31.2% chlorine were obtained. A 10% blend of this product in a mineral lubricating oil of 45 seconds vis. at 210° F. carried a full shock load of 15 weights in the Almen test as compared with 3 weights carried by the straight mineral oil. The reaction product in this example may be appropriately described as a piperidyl dithioformic chloroalkyl ester where the ester-forming group is chlorinated kerosene. As previously indicated, this group may be a halogenated paraffin wax or a halogenated aromatic petroleum fraction instead of kerosene is desired.

#### EXAMPLE 2

20 parts by weight sodium hydroxide  
42.5 parts by weight carbon disulfide  
25 78.7 parts by weight diamyl amine  
407 parts by weight chlorinated kerosene containing 39.8% of chlorine

The carbon disulfide was reacted with the caustic and amine in the same manner as described in Example 1, resulting in a clear yellow solution which was then refluxed with the chlorinated kerosene for 2 hours and the product isolated. 485 parts by weight of a product containing 5.3% of sulfur and 28.6% chlorine was obtained. A 10% blend of this product in mineral lubricating oil carried a full shock load of 15 weights in the Almen test. The composition thus formed may be considered to be a diamyl dithiocarbamic chloroalkyl ester where the ester-forming group is chlorinated kerosene. Instead of chlorinated kerosene, as previously indicated, halogenated paraffin wax or halogenated aromatic petroleum fractions may be used. More specifically, a chlorinated pentadecyl hydrocarbon may be used in lieu of or as a part of the chlorinated kerosene in which case the reaction product would comprise or consist of diamyl dithiocarbamic pentadecyl ester.

#### EXAMPLE 3

20 parts by weight sodium hydroxide  
43.5 parts by weight carbon disulfide  
62.1 parts mixed xylylidines  
405 parts of chlorinated kerosene containing 39.8% of chlorine

The caustic, xylylidines and carbon disulfide were reacted in the presence of methyl ethyl ketone as described in Example 1, yielding a heavy yellow suspension which was refluxed with the chlorinated kerosene in methyl ethyl ketone. After removal of the solvent and inorganic salts, 449 parts of a product containing 3.4% sulfur and 30.4% chlorine was obtained. A blend of 10% of this product in mineral lubricating oil (45 vis. at 210° F.) carried a full shock load of 15 weights in the Almen test. As in Examples 1 and 2 above, other halogenated hydrocarbons may obviously be substituted for chlorinated kerosene.

70 To illustrate the improved corrosion characteristics of the compounds of the present invention, 10% blends of these products in a highly refined mineral lubricating oil (45 seconds vis. at 210° F.) were made up and tested according to the following procedure. 200 cc. of the blend

and 2 cc. of water were vigorously agitated for 3 minutes. A Timken cup and an Almen pin were then placed in the lubricant and the lubricant stored in an oven at 120° F. for 48 hours at which time the extent of corrosion was noted. The results of these tests are shown in the following table.

Table

|                                                                       | Extent of corrosion | 10 |
|-----------------------------------------------------------------------|---------------------|----|
| Lubricating oil+10% commercial extreme pressure additive <sup>1</sup> | Marked              |    |
| Lubricating oil+10% of the product made in Example 1                  | Very slight         | 15 |
| Lubricating oil+10% of the product made in Example 2                  | Slight stain        |    |
| Lubricating oil+10% of the product made in Example 3                  | Slight stain        |    |

<sup>1</sup> Commercial extreme pressure additive containing sulfur and chlorine, but no nitrogen.

What is claimed is:

- As a composition of matter, piperidyl dithiocformic chloro-alkyl ester, where the ester-forming group is chlorinated of 5 to 50% chlorine content by weight kerosene.
- As a composition of matter, a product hav-

ing the general formula XCSSR'Hal<sub>x</sub>, in which X is selected from the group consisting of piperidine and radicals RR'N, R being a hydrocarbon radical selected from the group consisting of alkyl, cycloalkyl, aryl, alkaryl, and aralkyl substituents and R' being selected from the group consisting of hydrogen, alkyl, cycloalkyl, aryl, alkaryl and aralkyl substituents; R'' is a hydrocarbon radical selected from the group consisting of kerosene and wax, x is a positive number of sufficient magnitude to make the halogen equal to from 5 to 40 weight per cent of the molecule.

3. As a composition of matter, diamyl dithiocarbamic chloroalkyl ester, wherein the ester forming group is chlorinated kerosene of 5 to 50% chlorine content by weight.

HARRY W. RUDEL.

#### REFERENCES CITED

The following references are of record in the file of this patent:

#### UNITED STATES PATENTS

| Number    | Name          | Date          |
|-----------|---------------|---------------|
| 2,396,487 | Blake         | Mar. 12, 1946 |
| 2,404,446 | Lieber et al. | July 23, 1946 |
| 2,491,772 | Rudel         | Dec. 20, 1949 |